

Patented July 20, 1926.

1,592,994

## UNITED STATES PATENT OFFICE.

JOHN R. TOWNSEND, OF BROOKLYN, NEW YORK, ASSIGNOR TO WESTERN ELECTRIC COMPANY, INCORPORATED, OF NEW YORK, N. Y., A CORPORATION OF NEW YORK.

### METALLIC COMPOSITION.

No Drawing.

Application filed May 26, 1923. Serial No. 641,747.

This invention relates to contact metals, and its object is an alloy for electrical contacts which combines resiliency with durability and which will reduce to a minimum the possibility of arcing upon the approach or separation of the contacts.

Ordinary wiping contacts are very subject to wear, and accordingly tend to become abraded. In this condition the tendency for an electrical arc to form just previous to and directly after contact is made is greatly increased. This arcing is not only deleterious in itself, but it tends to erode the contacts still further, making them more subject to wear and to arcing. The deterioration of contacts under such conditions is therefore rapid.

This invention provides contact members which are abraded but little when wiping contact is made therebetween, and by their use the ordinary wear and arcing of the contact members and their subsequent rapid deterioration is avoided. To this end the contact members are formed of a phosphor-bronze to which a small portion of lead has been added; for example, a metallic composition containing the following ingredients: tin 4 to 5½%, lead 1 to 4%, phosphorus .05 to .25%, copper remainder.

Such a composition has the necessary resiliency for use in spring contacts and is

also sufficiently resistant to the effects of wear to provide wiping contact members which will be subject to arcing and deterioration in an unusually small degree. Wiping springs made of this material, for instance, show little effects of wear even after five million wiping make and break operations, whereas bronze wiping springs are useless after three million operations. Contact members formed of the same materials as above, but in different proportions, have also proved exceedingly satisfactory.

The invention claimed is:

1. An electrical contact element composed of phosphor-bronze alloy and lead, the amount of lead being in slight excess of its solubility.

2. A wiping contact member composed of a phosphor bronze alloy containing an amount of lead in slight excess of its solubility and at least as small as 4%.

3. A resilient contact member composed of a metallic composition containing the following metals in substantially the following proportions: tin 4 to 5½%, lead 1 to 4%, phosphorus .05 to .25%, and copper, remainder.

In witness whereof, I hereunto subscribe my name this 24th day of May A. D., 1923.

JOHN R. TOWNSEND.